

April 3, 1934.

S. A. PECK

1,953,310

PACKAGE BINDER

Filed Dec. 26, 1931

*Fig. 1.*



*Fig. 2.*



*Fig. 3.*



*Fig. 4.*



*Fig. 6.*



*Fig. 5.*



*Inventor:*

Samuel A. Peck  
By William A. Bradbury,  
McCaleb & Kinke, Attoys.

## UNITED STATES PATENT OFFICE

1,953,310

## PACKAGE BINDER

Samuel A. Peck, Cleveland, Ohio, assignor to Sig-node Steel Strapping Company, Chicago, Ill., a corporation of Delaware

Application December 26, 1931, Serial No. 583,329

14 Claims. (Cl. 91—68)

This invention relates to package binders and particularly to binders which are intended to be employed in binding packages, either individual packages or an assembly of packages.

- 5 In the normal use of such binders, the binder is applied around the package or assembly of packages and is tensioned by suitable devices, whereafter the ends of the binder are secured together in suitable manner. During the tensioning the binder bears upon the corners or other projecting portions of the packages and slides thereover with very great pressure. In certain well known forms of tensioning devices employed in connection with strap binders, portions
- 10 of the strap are located in superposed relation between gripping surfaces which apply a considerable pressure upon the straps. One of these gripping surfaces is adapted to be moved so as to apply considerable tension to the strap
- 15 and to cause one strap to slide over the other. Examples of such stretching or tensioning tools are illustrated in United States patents to Flora, No. 1,149,569, dated August 10, 1915 and to Guenther, No. 1,453,564, dated May 1, 1923.
- 20 In order to secure the superposed portions of the strap together, they are deformed in suitable manner with or without a sleeve being applied thereto, this operation being termed the sealing step. In a well known form of seal the straps are crimped together laterally so as to provide them with complementary inclined surfaces which oppose relative movement between the straps in the longitudinal direction. These
- 25 surfaces are formed with relatively slight movement between the contiguous surfaces of the straps. Examples of such seal-joints are illustrated in United States patents to Flora, No. 1,252,680 dated January 8, 1918 and to Leslie, No. 1,445,330, dated February 13, 1923.
- 30 One of the objects of the invention is to provide a strap having a normally high coefficient of friction so as to materially improve the efficiency of the engagement between the strap surfaces in such a seal.
- 35 A further object of the invention is to provide an improved binder having a surface coating which effectively protects the binder against corrosion.

A further object of the invention is to provide a binder having a coating which has a normally high coefficient of friction and which is adapted to break down when subjected to slippage under high pressure so as to substantially lower its coefficient of friction.

55 A further object of the invention is to provide

a binder having a coating which has a normally high coefficient of friction, which is capable of withstanding relatively slight slippage without effecting said coefficient of friction, and which is adapted to break down under the action of 60 slippage under high pressure so as to substantially reduce its coefficient of friction.

Other objects, advantages, and capabilities of the invention will hereinafter appear from the following description of preferred embodiments 65 of the invention, taken in conjunction with the accompanying drawing, in which:

Figure 1 is a sectional view of a strap embodying my invention, on an enlarged scale;

Fig. 2 is a plan view showing the overlapping 70 straps secured together by a seal of known type;

Fig. 3 is an elevation thereof;

Fig. 4 is a sectional view taken on the line 4—4 of Fig. 3;

Fig. 5 is a sectional view taken on the line 5—5 75 of Fig. 3; and

Fig. 6 is a sectional view of a wire binder embodying the invention.

In accordance with the invention I provide a steel strap 10 with a coating 11 of a suitable material having a surface of substantial coefficient of friction. This coating encloses particles of solid lubricating material 12.

Among the materials of which I may form the coating 11 are lacquers, varnishes, and dried oils. 85 I may form the coating from natural or artificial drying oils. I prefer, however, to employ a suitable mineral oil which is dried by heat treatment so as to leave a residue providing a protective coating having the desired high coefficient of friction. To obtain this result, I prefer to employ a crude asphalt base oil and have obtained excellent results with such an oil having a specific gravity about 0.94.

Among the solid lubricants which I may employ 95 I might mention talc and graphite. The solid lubricant is mixed with the coating material in its initial liquid state and is preferably in finely divided condition. I have obtained excellent results by using deflocculated graphite.

In order to facilitate complete understanding of the invention I give the following specific example. An asphalt base crude oil having a specific gravity of 0.9434 normally used as a coloring oil in steel finishing, was mixed with a commercial 105 concentrated colloidal suspension of graphite in a crude oil so as to produce a mixture containing approximately 0.1% of graphite. The steel strap was passed through a bath of this mixture and excess liquid was removed from the strap by wip- 110

ers or brushers. The strap was then passed through a muffle furnace in which it was subjected to a temperature of about 1100° for about forty seconds. This treatment completely dried the oil by the evaporation of all volatile matter with a minimum of oxidation. The strap, in finished condition, had a coating of dry, hard, brown residue which had a thickness of about 5/10000 of an inch. The surface of this coating possessed a coefficient of friction substantially higher than that of steel straps finished in the normal way. The particles of graphite were sealed within the coating and had no apparent effect upon the coefficient of friction of its surface.

15. Wire binders such as shown at 13 may be coated in the same way, the coating and solid lubricant particles being indicated by the same reference numerals in this figure.

In the form of seal illustrated in Figs. 2, 3 and 20 4 the overlapping portions of the strap 10 have applied thereto a clip 14 which is provided with flanges 15 which extend below the lower strap. At two intermediate positions, the clip 14 and the straps are deformed by suitable sealing machines 25 in the manner shown in Fig. 5. The center of the clip and the portions of the strap engaged thereby are substantially undeformed, as will readily be seen in Fig. 4. From a comparison of Figs. 4 and 5 it will immediately be understood that there 30 is substantially no slippage during the sealing operation between the contiguous strap surfaces and between the outer strap surfaces and the contiguous surfaces of the clip. Consequently the strap coating is not broken down at the sealing 35 position and the high coefficient of friction provided by my improved coating is undisturbed. In particular it is to be noted that there is no slippage whatever in the arched portion 16 of the seal and it is here that the maximum friction is obtained.

40. The high coefficient of friction provided by my improved coating enhances the frictional resistance provided by these inclined surfaces so as to result in a much more satisfactory seal than has been heretofore obtained with ordinary straps.

45. As heretofore explained, when the strap is subjected to substantial slippage under high pressure, for example in contact with the corners or projecting portions of the package, or in certain types of stretching machines, the coating breaks down 50 and the solid lubricant is liberated, thereby facilitating tensioning and insuring a more equal condition of tension throughout the length of the strap.

In the case of wire bindings, substantially the 55 same advantages are obtained. Wire bindings are ordinarily secured together by twisting operations which involve little or no relative movement between the contacting surfaces of the twisted wire. Consequently the high coefficient of friction of 60 these surfaces is preserved, thus providing a more satisfactory tying. At the corners of packages and other positions where the wire is subjected to substantial pressure and slippage, the coating breaks down and the liberated solid lubricant facilitates the movement of the wire.

Although the invention has been disclosed in connection with the specific details of preferred embodiments thereof, it must be understood that such details are not intended to be limitative of 70 the invention, except insofar as set forth in the accompanying claims.

Having thus described my invention, what I claim as new and desire to protect by Letters Patent is:

75. 1. A metal binder for packages having a pro-

tective coating of high coefficient of friction, said coating being adapted to break down when subjected to substantial slippage under high pressure, and solid lubricant distributed in said coating adapted to be liberated, when the coating breaks down, in sufficient quantity to provide the binder with a low coefficient of friction.

2. A metal binder for packages having a protective coating of high coefficient of friction, and solid lubricant particles enclosed within said coating, said coating being adapted to break down when subjected to slippage under high pressure to liberate said particles and said particles being present in sufficient quantity to provide the broken down coating with a low coefficient of friction.

3. A metal binder for packages having a coating of dried oil of high coefficient of friction and solid lubricant particles distributed within said coating in sufficient quantity to render the coating, when broken down by abrasion, of low coefficient of friction.

4. A metal binder for packages having a hard residual asphaltic coating of high coefficient of friction, and solid lubricant particles distributed 100 within said coating.

5. A metal binder for packages having a coating of dried oil of high coefficient of friction and solid graphite particles distributed within said coating in sufficient quantity to render the coating, when broken down by abrasion, of low coefficient of friction.

6. A metal binder for packages having a hard residual asphaltic coating of high coefficient of friction, and solid graphite particles distributed 110 within said coating.

7. The method of coating a metal binder for packages which comprises adding finely divided solid lubricant to a liquid coating material, coating the binder with the mixture, and drying the 115 liquid material to produce a surface of high coefficient of friction, said solid lubricant being added in sufficient quantity that it imparts a low coefficient of friction to the coating when broken down by abrasion.

8. The method of coating a metal binder for packages which comprises adding finely divided graphite to a liquid coating material, coating the binder with the mixture, and drying the liquid material to produce a surface of high coefficient 125 of friction, said graphite being added in sufficient quantity that it imparts a low coefficient of friction to the coating when broken down by abrasion.

9. The method of coating a metal binder for 130 packages which comprises adding a suspension of deflocculated graphite to a liquid coating material, coating the binder with the mixture, and drying the liquid material to produce a surface of high coefficient of friction, said deflocculated 135 graphite being added in sufficient quantity that it imparts a low coefficient of friction to the coating when broken down by abrasion.

10. The method of coating a metal binder for packages which comprises adding finely divided 140 solid lubricant to asphaltic base oil, coating the binder with the mixture, and drying the applied material to leave a hard residual coating of high coefficient of friction, said solid lubricant being added in sufficient quantity that it imparts a low 145 coefficient of friction to the coating when broken down by abrasion.

11. The method of coating a metal binder for packages which comprises adding finely divided graphite to asphaltic base oil, coating the binder 150

- with the mixture, and drying the applied material to leave a hard residual coating of high coefficient of friction, said graphite being added in sufficient quantity that it imparts a low coefficient of friction to the coating when broken down by abrasion. 5
12. The method of coating a metal binder for packages which comprises adding a suspension of deflocculated graphite to asphaltic base oil, coating the binder with the mixture, and drying the applied material to leave a hard residual coating of high coefficient of friction, said deflocculated graphite being added in sufficient quantity that it imparts a low coefficient of friction to the coating when broken down by abrasion. 10
13. A metal binder for packages having a hard residual asphaltic coating of high coefficient of friction, and solid lubricant particles distributed within said coating in sufficient quantity to provide the coating with a low coefficient of friction when it is broken down by abrasion. 80
14. A metal binder for packages having a hard residual asphaltic coating of high coefficient of friction, and solid graphite particles distributed within said coating in sufficient quantity to render the coating, when broken down by abrasion, of low coefficient of friction. 85

SAMUEL A. PECK. 90

|    |     |
|----|-----|
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |